

# United States Patent Office

3,372,977

Patented Mar. 12, 1968

1

3,372,977

## PROCESS OF CREESEPROOFING CELLULOSIC TEXTILES WITH A SINGLE AQUEOUS SOLUTION CONTAINING BOTH D,1-BUTADIENE DIOXIDE AND A LEWIS BASE CATALYST

Ralph J. Berni, Ruth R. Benerito, and John B. McKelvey, New Orleans, La., assignors to the United States of America as represented by the Secretary of Agriculture No Drawing. Filed Aug. 27, 1965, Ser. No. 483,372  
1 Claim. (Cl. 8—120)

A non-exclusive, irrevocable, royalty-free license in the invention herein described, throughout the world for all purposes of the United States Government, with the power to grant sublicenses for such purposes, is hereby granted to the Government of the United States of America.

This invention relates to the production of cellulosic textiles with improved crease recovery characteristics. More specifically this invention relates to the production of cellulosic fabrics with improved dry and wet crease recovery characteristics imparted through etherification of the cellulose hydroxyl groups when reacted with d,1-butadiene dioxide, which is structurally represented by the formula



and various Lewis bases in aqueous media. Utility of the present invention is found in the fact that the cellulosic fabrics produced by process of this invention show improved dry and wet crease recovery without unduly altering the strength, hand, or appearance of the finished fabric.

The primary object of the invention is to produce butadiene diepoxide etherified cotton fabrics exhibiting improved crease recovery properties by means of an all aqueous treatment. Prior art processes utilized 2- or 3-phase systems to produce crease resistant fabrics. Practical processes utilizing all-aqueous systems are preferred in commercial processes over nonaqueous systems.

Another object of this invention is to provide a process for etherifying cotton fabrics with butadiene dioxides, which can produce fabrics with moderate increases of dry crease recovery, for example, those in the 240° to 250° (W plus F) range; and moderate to large increases in wet recovery, for example, those in the 240° to 280° (W plus F) range. Prior art processes have produced excessive increases in crease recovery, which have proved to be unfavorable in subsequent garment cutting operations.

A third object of this invention is to provide an etherification process which utilizes general base catalysis, since combined processes (dyeing, softening, calendering, etc.) involve restrictions in use of strong caustic solutions, therefore weaker bases are indicated.

In general, according to our present invention a cellulosic material, such as cotton (0.06 mole), is reacted by immersing for a period of time about from 10 minutes to 24 hours in a solution containing about from 0.125 to 0.250 mole of butadiene dioxide and sufficient water to make 100 ml., and catalyzed with about from 0.01 to 0.03 mole of a Lewis base selected from the group consisting of sodium hydroxide, potassium hydroxide, lithium hydroxide, ammonium hydroxide, aniline, pyridine, piperidine, morpholine, quinoline, cyclohexylamine, 2-amino-pyridine, 3-aminopyridine, 4-aminopyridine, 3-pyridol, monoethanolamine, diethanolamine, and triethanolamine,

2

and a cotton fabric which possesses improved wet and dry crease resistance is obtained. The applicable molar ratios are about from 1:2.16 to 1:4.50, anhydroglucose units of cellulose to butadiene dioxide to catalyst, respectively.

Prior art processes required more expensive nonaqueous systems for producing dry and wet crease recovery on cotton using d,1-butadiene dioxide in basic or acidic media. Our present invention takes advantage of the surface polymerization as well as the crosslinking mechanisms to obtain products which produce improved dry and wet recovery for cotton cellulose at room temperature.

The term Lewis base is defined as any molecule or ion having unshared electron pairs available for sharing with acids. All of the bases mentioned in this application are included in this classification, and all catalyze the etherification (cellulose-butadiene dioxide reaction) with varying degrees of efficiency.

The preferred method for obtaining the desired results consists in complete immersion of an 80 x 80 or a 68 x 72 cotton fabric into a container filled with 100 ml. of an aqueous solution containing from 0.125 to 0.250 mole of d,1-butadiene dioxide, and from 0.01 to 0.03 mole of a catalyst or coreactant Lewis base, and reacted at ordinary room temperature (20° to 30° C.) for a period of from about 10 minutes to 24 hours. The sequence of solution preparation is critical in that the water and butadiene dioxide must be first combined before addition of the catalyst since the addition of catalyst to the concentrated epoxide would cause rapid polymerization thereby destroying the reaction media. After the etherified cotton is removed from the reaction vessel the fabric is quenched in a weakly acidic solution, washed in tap water, and distilled water, and ironed dry. The fabric obtained exhibits increased dry (conditioned) and wet recovery without surrendering its basic fabric properties.

Dry crease recovery evaluations are expressed in degrees, are a summation of Warp and Filling, and were done according to U.S. Federal Supply Service, Federal Specification CCC-T-191b, Method 5212, Washington, D.C., U.S. Government Printing Office (1951), while the wet crease recovery evaluations were determined by a method described by R. A. Fujimoto, R. M. Reinhardt, and J. D. Reid in the American Dyestuff Reporter, 52, P329 (1963).

The examples set forth are meant to illustrate the practice of our present invention, and are not meant to be construed as limiting the invention in any manner whatever.

### Example 1

A 10.0 gm. sample of 68 x 72 cotton fabric (0.06 mole) was rolled and placed in a 100 ml. graduated cylinder containing 20 ml. of d,1-butadiene diepoxide (0.25 mole) and 130 gm. of NaOH (0.03 mole) diluted with distilled water to 100 ml. The fabric was allowed to remain immersed and react for 24 hours. The fabric sample was then removed from the solution, rinsed in methanol, neutralized with aqueous acetic acid, and quenched in tap water for at least 15 minutes, then ironed dry. The treated fabric sample had a weight add-on of 8.3%; and the dry and wet crease angles were respectively 254° and 289° (W plus F).

### Example 2

Eight 10.0 gm. (0.06 mole) samples of cotton fabric were treated by the process of Example 1 and in a solution of the same composition except that eight different

reaction times were employed. The significant data are shown in Table I.

and molecular quantities used in the reaction, and results of significance to this invention.

TABLE II

| Fabric Sample (No.) | Reagent              | Quantity (moles) | RESULTS          |                 |
|---------------------|----------------------|------------------|------------------|-----------------|
|                     |                      |                  | Add-On (Percent) | Crease Recovery |
|                     |                      |                  | Dry              | Wet             |
| 4                   | Aniline              | 0.02             | 4.0              | 207 169         |
| 5                   | Morpholine           | 0.01             | 5.6              | 227 249         |
| 6                   | do                   | 0.02             | 6.8              | 237 256         |
| 7                   | Piperidine           | 0.01             | 6.0              | 230 249         |
| 8                   | do                   | 0.02             | 8.0              | 226 278         |
| 9                   | Quinoline            | 0.01             | 2.6              | 211 217         |
| 10                  | do                   | 0.02             | 3.7              | 218 234         |
| 11                  | Cyclohexylamine      | 0.01             | 3.7              | 228 235         |
| 12                  | do                   | 0.02             | 5.9              | 229 238         |
| 13                  | Benzylidimethylamine | 0.01             | 5.5              | 227 246         |
| 14                  | do                   | 0.02             | 7.6              | 248 274         |
| 15                  | 2-aminopyridine      | 0.01             | 3.9              | 241 228         |
| 16                  | 3-aminopyridine      | 0.01             | 6.2              | 256 253         |
| 17                  | 4-aminopyridine      | 0.01             | 6.0              | 246 237         |
| 18                  | 2-pyridol            | 0.01             | 3.4              | 244 218         |
| 19                  | Pyridine             | 0.01             | 8.9              | 243 270         |
| 20                  | do                   | 0.02             | 9.8              | 227 259         |
| 21                  | $\alpha$ -Picoline   | 0.01             | 7.2              | 218 248         |
| 22                  | do                   | 0.02             | 9.2              | 221 267         |
| 23                  | Monothanolamine      | 0.02             | 5.7              | 230 236         |
| 24                  | Diethanolamine       | 0.01             | 4.7              | 225 231         |
| 25                  | Triethanolamine      | 0.01             | 3.7              | 209 230         |

TABLE I

| Fabric Sample No.    | Reaction Time (minutes) | Results          |                                                         |     |
|----------------------|-------------------------|------------------|---------------------------------------------------------|-----|
|                      |                         | Add-On (percent) | Crease Recovery Angles (degrees, W plus F) <sup>1</sup> |     |
|                      |                         |                  | Dry                                                     | Wet |
| a                    | 10                      | 0.33             | 185                                                     | 206 |
| b                    | 20                      | 1.28             | 191                                                     | 209 |
| c                    | 30                      | 2.80             | 182                                                     | 223 |
| d                    | 50                      | 6.39             | 225                                                     | 277 |
| e                    | 70                      | 8.25             | 234                                                     | 281 |
| f                    | 80                      | 8.71             | 231                                                     | 278 |
| g                    | 90                      | 9.23             | 224                                                     | 271 |
| h                    | 180                     | 8.11             | 229                                                     | 286 |
| Control <sup>2</sup> |                         |                  | 180                                                     | 180 |

<sup>1</sup> Crease recovery values are a summation of Warp and Filling angles, 40 and are expressed in degrees.

<sup>2</sup> Untreated sample.

### Example 3

45

A 10.0 gm. (0.06 mole) sample of 68 x 72 cotton fabric was treated by the process of Example 1 except that aqueous ammonium hydroxide (0.030 mole) was used instead of aqueous sodium hydroxide to obtain a fabric with 7.6% add-on, and the dry and wet crease angles were respectively 260° and 241° (W plus F).

### Examples 4 through 25

55

Twenty-four 10.0 gm. (0.06 mole) samples of 68 x 72 cotton fabric were treated by the process of Example 1 except that an aqueous amine was used instead of aqueous sodium hydroxide. Table II shows the various amine

We claim:

1. A process for imparting improved wet and dry crease recovery to cellulosic textile comprising reacting cellulosic textile containing free cellulose hydroxyl groups by immersing said textile in an aqueous solution consisting essentially of d,1-butadiene dioxide and a Lewis base catalyst in molar ratio of from about 1:2:0.16 to 1:4:0.50, respectively of anhydroglucose units of cellulose:d,1-butadiene dioxide:catalyst, for a period of time from about 10 minutes to 24 hours at room temperatures, said aqueous solution being produced by dissolving the d,1-butadiene dioxide in water and then adding said catalyst.

### References Cited

#### UNITED STATES PATENTS

- 3,150,920 9/1964 Berni et al. \_\_\_\_\_ 8—120  
3,268,293 8/1966 McElvey et al. \_\_\_\_\_ 8—120

#### OTHER REFERENCES

- Journal of Polymer Science, vol. 51, pp. 209—230 (1961) 8/120.  
Journal of Polymer Science, part A, vol. 1, pp. 3407—3426 (1963) 8/120.  
50 Textile Research Journal, February 1963, pp. 117—129 8/120.  
Journal of Polymer Science, vol. 9, pp. 181—190 (1965) 8/120.  
55 Journal of Polymer Science, vol. 9, pp. 191—205 (1965) 8/120.

NORMAN G. TORCHIN, Primary Examiner.

H. WOLMAN, Assistant Examiner.